

## UNITED STATES PATENT OFFICE

2,047,278

## PROCESS FOR THE FIBROUS ESTERIFICATION OF CELLULOSE

Carl J. Malm, Rochester, N. Y., and Charles L. Fletcher, Kingsport, Tenn., assignors to Eastman Kodak Company, Rochester, N. Y., a corporation of New York

No Drawing. Application May 19, 1933,  
Serial No. 671,901

9 Claims. (Cl. 260—101)

The present invention relates to a fibrous process of esterifying cellulose in which a liquid saturated hydrocarbon is employed as the non-solvent and chlorinated hydrocarbon is employed to homogenize the ingredients of the esterification bath.

Among the most effective non-solvents yet employed in the fibrous esterification of cellulose are the saturated hydrocarbons either aliphatic such as hexane or heptane or cyclic such as cyclohexane.

Some of the hydrocarbon non-solvents which are suitable in fibrous esterification processes are known under various names such as ligroin, petroleum ether, Stoddard solvent, kerosene, gasoline, naphtha, etc. Stoddard solvent is a commonly known aliphatic hydrocarbon which is described in "Bureau of Standards Bulletin CS 3—28 (1929)." In the fibrous processes where these saturated hydrocarbons are employed as the non-solvents in the esterification of cellulose the amounts necessary to assure insolubility of the resulting ester in the esterification bath are much less than is the case with the non-solvents which are ordinarily employed. However these non-solvents suffer the disadvantage that their mixtures with the lower fatty acids and anhydrides are heterogeneous especially in those cases where hydrocarbons having a high boiling range are employed.

One object of our invention is to provide a process for the fibrous esterification of cellulose in which a saturated hydrocarbon may be employed as the non-solvent and yet the bath is homogeneous and from which the non-solvent and homogenizing liquid may be easily removed after the completion of the esterification. Another object of our invention is to provide a fibrous process for the esterification of cellulose in which the recovery of the individual ingredients is facilitated.

The broad idea of employing a homogenizer in conjunction with a saturated hydrocarbon in the fibrous esterification of cellulose is the invention of Minsk, Kenyon and Gray and is disclosed and claimed in their application Serial No. 671,900, filed of even date. We have found that if certain chlorinated hydrocarbons are employed in a fibrous esterification bath in which a saturated hydrocarbon is the non-solvent, the separation and recovery of the ingredients of the spent esterification bath is greatly facilitated. We have found that the halogenated hydrocarbons are especially suitable as homogenizers in fibrous esterification processes, as they may re-

place the fatty acid ordinarily employed in an esterification mixture and they form an azeotropic constant boiling mixture with water. We have found that by our invention many of the difficult and often unsatisfactory methods of recovering the ingredients of a spent fibrous esterification bath are eliminated which have been heretofore thought necessary or at least preferable in such recovery.

In a fibrous esterification process in which a saturated hydrocarbon is employed as the non-solvent, a surprisingly small amount of that hydrocarbon is necessary to render the esterification bath non-solvent of the cellulose ester formed, in fact, the non-solvency of this liquid is so pronounced that it extends even to the constituents of the esterification bath. By the present invention the effectiveness of the saturated hydrocarbon to induce non-solvency of the cellulose ester by the esterification bath may be utilized and an even esterification of the cellulose may be assured.

The halogenated hydrocarbons when employed as homogenizers also present other advantages in addition to those pointed out above. Many of them are inflammability reducing agents which feature is very valuable in case of the more volatile hydrocarbons such as gasoline or the like. For instance a mixture of 50 parts of trichlorethylene and 50 parts of Stoddard solvent is totally non-inflammable. Even in the case of a halogenated hydrocarbon such as ethylene chloride which will burn, that material has a comparatively high flash point so that the danger of ignition is much less compared with some of the other homogenizers which might be employed. The halogenated hydrocarbons are excellent solvents for the ingredients of the esterification bath and in the case of some of these hydrocarbons such as ethylene chloride the amount required for homogenizing is less than that required when using some other homogenizing liquid. We have found that ethylene chloride, propylene chloride and trichlorethylene are the most satisfactory in our invention however other chlorinated hydrocarbons such as methylene chloride, carbon tetrachloride, chloroform or other halogenated hydrocarbons may be employed with marked success.

The bromide, iodide and fluoride compounds which correspond to the chlorinated hydrocarbons would also be suitable for homogenizing esterification baths which would otherwise be heterogeneous.

Our process comprises the esterification of cellulose in a bath comprising a fatty acid anhy-

dride, a saturated hydrocarbon as the non-solvent, an azeotrope-forming chlorinated hydrocarbon as the homogenizer and a catalyst such as perchloric or sulfuric acid.

5 When the esterification is completed, the recovery of the spent esterification bath may be carried out as follows:

The liquid is removed from the fibrous ester formed, by centrifuging. The cellulose ester now 10 contains less than an equal weight of liquid which consists of the non-solvent, the chlorinated hydrocarbon, a small quantity of fatty acid and the catalyst. The ester is then placed in a vessel adapted for steam distillation and water and a 15 sufficient quantity of sodium carbonate to neutralize the catalyst is added. The chlorinated hydrocarbon and the non-solvent may be removed by steam distillation. The quantity of fatty acid remaining is negligible and may be 20 economically discarded. The ester is washed with water to remove the fatty acid and sodium salt and may then be dried.

The following examples illustrate processes which embody our invention:

25 *Example I*

30 lbs. of cotton linters were added to a mixture of 90 lbs of Stoddard solvent, 90 lbs. of acetic anhydride, 120 lbs. of ethylene chloride and 810 c. c. of a catalyst consisting of 3 parts by volume of phosphoric acid and 1 part by volume of sulfuric acid all at a temperature of 70° F. The mixture was stirred occasionally and the temperature in the jacket of the reaction vessel 35 was raised uniformly to a temperature of 120° F. over a period of 4 hours. The mass was maintained at that temperature until a washed and dried sample taken therefrom showed solubility in a mixture of 85 parts of chloroform and 15 40 parts of ethyl alcohol by volume. This usually requires 10-15 hours.

The fibers were then separated from the main portion of the reaction liquid by centrifuging. The remainder of the reaction liquid was removed from the fibers by adding water containing sufficient sodium carbonate to neutralize the catalyst, steam distilling out the ethylene chloride and Stoddard solvent and washing out the remaining acid with water. The product which 50 was a cellulose triacetate was dried in the usual manner.

*Example II*

30 parts of cotton linters were added to a solution consisting of 90 lbs. of Stoddard solvent, 55 120 lbs. of propylene chloride, 60 lbs. of 85% acetic anhydride, 45 lbs. of 94% propionic anhydride and 200 c. c. of sulfuric acid as the catalyst, all at a temperature of 70° F. The temperature in the jacket of the reaction vessel was 60 raised uniformly to 120° F. over a period of 4 hours and the temperature was maintained at this point until the product was soluble in a mixture of 90 parts of ethylene chloride and 10 parts of methyl alcohol by volume. The product, cellulose acetate propionate was processed 65 as in the preceding example to remove the reaction liquid therefrom.

Although the present invention will be ordinarily applicable to fibrous processes in which the 70 petroleum distillates are employed as the non-solvent, it is obviously applicable to the use of any non-solvent which renders the esterification bath heterogeneous thus necessitating the presence of a homogenizer to assure an even esterification. In these processes the fatty acid ordi-

narily employed may be entirely replaced by the halogenated hydrocarbon in accordance with our invention however if desired this substitution of halogenated hydrocarbon for fatty acid may be only partial and the process would still fall 5 within the scope of our invention.

It is to be understood that our invention is directed broadly to the preparation of organic acid esters of cellulose although as the simple and mixed esters of cellulose containing acetyl, 10 propionyl and butyryl groups are more common at the present time, our invention is more particularly directed to the preparation of cellulose esters containing one or more of those lower fatty acid groups. 15

We claim as our invention:

1. A process for preparing an organic acid ester of cellulose in fibrous form which comprises reacting upon the cellulose with an esterifying bath containing a liquid petroleum distillate which is essentially within a boiling range of 40-210° C. as the non-solvent and a halogenated hydrocarbon, in sufficient amount to assure compatibility of the ingredients of the bath, which bath will not dissolve the ester formed 25 therein.

2. A process for preparing an organic acid ester of cellulose in fibrous form which comprises reacting upon the cellulose with an esterifying bath containing a liquid petroleum distillate which is essentially within a boiling range of 40-210° C. as the non-solvent and a chlorinated hydrocarbon, in sufficient amount to assure compatibility of the ingredients of the bath, which bath will not dissolve the ester formed 35 therein.

3. A process for preparing an organic acid ester of cellulose in fibrous form which comprises reacting upon the cellulose with an esterifying bath containing a liquid petroleum distillate which is essentially within a boiling range of 40-210° C. as the non-solvent and a chlorinated olefine, in sufficient amount to assure compatibility of the ingredients of the bath, which bath will not dissolve the ester formed therein. 40

4. A process for preparing an organic acid ester of cellulose in fibrous form which comprises reacting upon the cellulose with an esterifying bath containing a liquid petroleum distillate which is essentially within a boiling range of 40-210° C. as the non-solvent and an alkylene chloride, in 50 sufficient amount to assure compatibility of the ingredients of the bath, which bath will not dissolve the ester formed therein.

5. A process for preparing an organic acid ester of cellulose in fibrous form which comprises 55 reacting upon the cellulose with an esterifying bath containing a liquid petroleum distillate which is essentially within a boiling range of 40-210° C. as the non-solvent and ethylene chloride, in sufficient amount to assure compatibility of the ingredients of the bath, which bath will not dissolve the ester formed therein.

6. A process for the preparation of cellulose acetate propionate in fibrous form which comprises reacting upon the cellulose with a bath 65 which contributes acetyl and propionyl groups to the cellulose and containing a liquid petroleum distillate which is essentially within a boiling range of 40-210° C. as the non-solvent and an alkylene chloride, in sufficient amount to assure 70 compatibility of the ingredients of the bath, which bath will not dissolve the ester formed therein.

7. A process for the preparation of cellulose acetate propionate in fibrous form which com- 75

- prises reacting upon the cellulose with a bath which contributes acetyl and propionyl groups to the cellulose and containing a liquid petroleum distillate which is essentially within a boiling range of 40-210° C. as the non-solvent and ethylene chloride, in sufficient amount to assure compatibility of the ingredients of the bath, which bath will not dissolve the ester formed therein.
- 10 8. A process for preparing an organic acid ester of cellulose in fibrous form which comprises reacting upon the cellulose with an esterifying bath containing a liquid petroleum distillate which is essentially within a boiling range of 40-210° C. as the non-solvent and propylene

chloride in sufficient amount to assure compatibility of the ingredients of the bath, which bath will not dissolve the ester formed therein.

9. A process for preparing an organic acid ester of cellulose in fibrous form which comprises reacting upon the cellulose with an esterifying bath containing a liquid petroleum distillate which is essentially within a boiling range of 40-210° C. as the non-solvent and trichlorethylene in sufficient amounts to assure compatibility of the ingredients of the bath, which bath will not dissolve the ester formed therein.

CARL J. MALM.  
CHARLES L. FLETCHER. 15